# EUROPEAN PATENT SPECIFICATION

(11) **EP 2 466 240 B1**
(45) Date of publication and mention of the grant of the patent: **20.11.2013**
(21) Application number: 11191029.5
(22) Date of filing: 28.11.2011
(51) Int. Cl.: F27B 17/00, F27D 1/16, F27D 1/18

(54) **Dry heating method of refractory ceramic construction**
Trocknungswärmeverfahren einer refraktiven Keramikkonstruktion
Procédé de séchage de construction de céramique réfractaire

(30) Priority: 17.12.2010 FI 20100422
(43) Date of publication of application: 20.06.2012
(73) Proprietor: Termorak Oy, 33880 Lempäälä (FI)
(72) Inventor: Pitkänen, Seppo, 33300 Tampere (FI)
(74) Representative: Gritschneder, Martin

(56) References cited:
- US-A- 4 304 986

## Description

The object of this invention is a dry heating method of a high temperature proof i.e. refractory ceramic lining. With the help of this method, the moisture of a refractory material construction is removed in a controlled way so that it does not damage the constructions when coming out. Likewise, by this method the temperature of a ceramic construction is raised so high that the temporary bonds of the construction, i.e. hydraulic bonds are removed in a controlled way and instead the final bonds i.e. ceramic bonds of the construction are formed. So by using the method, the moisture is removed from the ceramic lining and the temporary bonds change into permanent bonds in such a way that the lining is not damaged.

The term "dry heating" is generally in use when speaking of the preparation of taking in use of the equipment including refractory constructions. It is also used in the documents of this application and it includes the raising of the temperature of the construction to about 550-600°C. The first phase is to raise the temperature slowly to about 110 - 120°C and keeping it there so long that essentially all the so called free water in the construction evaporates and comes out from the construction in the form of steam. In the second phase, the temperature is raised in a controlled way and sufficiently slowly so high that the ceramic bonds of the construction are formed instead of the essentially out coming temporary hydraulic bonds. In this phase, the changes and structure of so called crystal water gets the greatest part of the final strength when the ceramic bonds are formed.

The before mentioned constructions are typically used in the industry boilers, gasifyer plants, industry kilns and corresponding plants. The parts that contain most water after the installation are made at the installation site of the refractory castable material that is made by mixing ceramic powder and water. The ceramic powder is typically made mainly of base material and bond material and can include also finer filler material. Alumina cement is used very often as a bond material. The material that is in the form that it can be casted or shaped is installed for example into molds where the hydraulic bond is formed when the water reacts with lime and the material hardens. After the molds have been removed and the air drying has taken place, the before mentioned drying heating is made for the construction before it is taken into use.

The making of the ceramic construction in the before mentioned equipments is performed either to the equipment that has been installed in the final placement location or to the parts of this equipment in a workshop before transporting them to the final location. The latter method is known to be the better way to install refractory linings, but it is not always possible because, for instance, it is sometimes very expensive and challenging to divide the pressurized body into certain sections. On the other hand, the plate frames, like for instance bio gasifiers, this is in many cases the more advantageous way to build the plants that have been refractory lined because a great part of the production can then be made in the advantageous workshop conditions and only the parts are put together at the installation site. And because of what has been said before, the dry heating must sometimes be done in the workshop or tent where the parts are produced and in some other cases at the installation site.

The before mentioned dry heating is performed nowadays in different ways depending on the conditions. The dry heating at the final place of the equipment especially in big plants is often performed using the own oil or gas burners of the plant burning them intermittently. The burner or burners like for instance the start-up burners of the fluidized bed boilers are used intermittently so that the inside temperature of the plant can be raised following as accurately as possible the temperature diagram for the drying heating. The process cannot be very accurate because it is not possible to fine tune using the burners. In fig 1 there is a typical temperature diagram for the dry heating of boilers or gasifiers, where the temperature is show as a function of time. There it can be seen that the temperature is first raised from the room temperature (20°C) to about 115 - 120°C with the speed of 20°C per hour. There are temperature detectors inside the lining or at the surface of it and they show when the lining is at this temperature all the way through and from that point on the temperature is kept for 8 hours, as the diagram says. Thereafter the burner efficiency is raised so that the raising speed of the temperature of the inside space or of the refractory lining is max 50°C per hour. It is advanced with this speed until the temperature of about 550°C has been reached which in turn is kept for 12 hours. The dry heating is now ready and the ceramic linings of the plant are ready to be taken into use. As an extension of the dry heating in a ready plant, the actual start-up run can be performed where the temperature of the plant is raised to the temperature of about 850 - 900°C.

The dry heating of smaller plants and plants to be made in parts is performed by prior-art technique by installing heating equipments to these plants and parts of plants. For instance the dry heating of the before mentioned bio gasifiers parts is made using the prior-art technique so that the open openings of the part are closed using means that are coated with ceramic fibre and the oil or the gas burner is put to an opening leading inside this package. The opening can be a part of the construction and then it can be for example a man hole or so, or it can be provided in parts that close the before mentioned openings. It is also taken care that there is an opening for out coming flue gas and steam. The power of the heating burner is regulated by hand and the temperature is monitored carefully during the whole process. When it is the question about for example a bio gasifier reactor section the outside diameter being 4 m, height 4 m and the thickness of the lining totaling 0.3 m, the section is put on the floor either on its side or upright and its open ends are equipped with before mentioned closing means (Fig 2). In one end a hole is made to the closing means for the boiler and to the other end closing means a hole is made for the flue gas and steam. As there is an isolating lining behind the cylinder surface lining, the cylinder itself does not need more lining for the dry heating. The burner like oil burner is put on and the own isolation of the section and the isolations in the closing means keep the warmth mainly inside the object and thus the inside temperature and the temperature of the lining start to rise. The flue gas goes out through the hole at the other end and it remains in the boiler house or is led out from it using canals. When the temperature of the lining has risen to 100°C the forming steam starts to get out together with the flue gas through the same hole. The power of the burner is increased during the drying heating within the limits of the drying diagram and the supervisor of the drying monitors all the time the temperatures and that the equipment function properly and removes and places new fuel vessels, like oil barrels or gas bottles.

The before described prior-art technique is used in the production of the applicant and its competitors.

The greatest disadvantages of the methods of the prior-art technique are the great costs it causes and it is impractical due to many reasons and low reliability of operation. In the dry heating of a section mentioned before the highest value of heating power is about 100 kW, the costs for the fuel according to today's price level is estimated about 5000 € and the cost for supervising the process is about 1500 - 2000 € (35 - 45 h). When the flue gas that contains a lot of energy is led out of the object and usually also out of the building where the dry heating is being done, means a big uneconomic factor. It is also uneconomic that the process must be monitored all the time for instance because of regulating the temperature and the fuel service and additionally there is a risk of fire and further there is necessity to eliminate malfunction of the equipment. A central factor that decreases the good function is the formation of steam inside the boiler house because this makes the air feeding to the boiler more difficult, the burning process becomes less sure and the burner is in danger to turn off by itself. Due to all this, it is difficult to follow the dry heating diagram and the heating schedule is drawn out easily. All this causes more energy and manpower costs. The process is more impractical because the lined parts get sooty and the flue gas comes into the boiler house.

This invention has as its objective to introduce such a dry heating method for ceramic linings that flaws in the prior-art technique can be avoided. The solution according to the invention is characterized in that what is presented in the patent claim 1 characterizing part.

The greatest advantages of the method according to the invention in comparison with the prior-art technique can be considered to be that the method according to the invention spares a lot of economical resources and the second point is that it is operational with great security. It is superiorly more practical in comparison with the prior-art technique. When the dry heating has been started it operates quite automatically without continuous monitoring and fuel service. In the method, no flue gases are formed so that the air inside the object can be directed to the inside circulation and, thus, also a considerable amount of energy is saved. The energy that is used in the process can now all in all be used more efficiently than what is possible in the prior-art technique applications. The method according to the invention is very clean and it does not cause sooty or otherwise unclean plant sections.

The invention is described more closely in the enclosed drawings, where:
Fig 1 presents one temperature diagram used in the drying heating, where the temperature is presented as a function of time;
Fig 2 presents a dry heating method with its equipments by the prior-art technique used in dry heating a gasifier section;
Fig 3 presents a section of the before mentioned bio gasifier in upright position equipped with equipments according to the invention of the dry heating system;
Fig 4 presents a cross section of the object of the previous fig 3 in the place marked in fig 3 A-A;
Fig 5 presents the blocking part like cover seen from the top;
Fig 6 presents the cross section of the before mentioned lid in the place B-B in fig 5, that is cut in the place of one electric resistance;
Fig 7 presents the down part of the temperature diagram where the principle of raising the
temperature is shown using the method according to the invention when performing the dry heating.

Now follows a description of an application of dry heating that is advantageous for the invention with the help of an example referring to figs that have been mentioned before.

In fig 3 there is a lined bio gasifier section placed in upright position on the floor of an industry hall. This position is also the final position of the section in the gasifier. The section is the object 100 of the dry heating. The outside diameter d of the object 100 is about 4 m and the height h also is about 4 m. Its shell 101 is bent steel sheet of 10 mm and inside it, a refractory ceramic lining 102 (fig 4) has been installed, and its total thickness is 300 mm. So the lining 102 has the shape of cylinder ring and it contains the outmost rings of isolating material 102a, 102b and the innermost ring 102c that is of tight refractory material casted at site. The rings 102a and 102b have been made of isolating sheet that has been cut to the shape of wedges and these pieces have been put together with mortar and the whole lining 102 has been anchored to the shell 101 using special anchors and it is supported downwards with a lining support shell 105. In this example, the isolation layers contain very little moisture because only the mortar that has been used in the installation contains a little water and the sheets itself are dry and thus their humidity is only what is caused by the humidity of the air. The innermost layer 102c in turn contains about 4 weight percent water. In this example, the thickness of the innermost layer 102c is 70 mm and the density of the material is 2,3 kg/dm³, so the ceramic lining 102 of this object 100 has received about 300 I water during the installation. A part of this water is free water that is removed in the form of steam during the dry heating and a part is crystal water in the lattice of the salts of the ceramic construction.

The dry heating system according to the invention operates in the before mentioned situation so that on the floor 103 of the hall, a platelike closing means 1 is placed that has been lined with 100 mm of high temperature resistant isolating fibre layer. The fibre is on top and upon it, a refractory lined object section 100 is lifted using a crane and thus the opening that points downwards, the first opening 104a, gets closed. On top of the object 100 a lid is lifted, that is the second closing means 2 and the surface of it that points towards the object 100 has been lined 100 mm thick using ceramic fibre layer 2a that is high temperature resistant and isolating and thus the upwards opening of the object 100, that is the second opening 104b, gets closed. The second closing means 2 is placed to its place so that the joint between the object 100 and the fibre layer of the second closing means 2 is tight. In the second closing means 2 and its fibre layer 2a there are many holes with diameters about 60 - 70 mm. A part of the holes that is the first holes 3 (fig 5) are located in the middle section of the second closing means 2 and a part of the holes that is holes 4 are in the edge area of the second closing means 2. The second closing means 2 consists of steel stiffeners 106 so that it is possible to work standing on it. There are total 12 first location holes 3 in an object 100 of the size of this example and an electric resistance 5 is installed in every one of them. The electric resistance is presented in more detail in fig 6. The electric resistance 5 consists of about 2 meters long oblong loop 5a, base 5b and connection cable 5c. The loop 5a consists of a tube like surface part and inside it there is a resistance wire. The material of it is for instance acid proof or fire proof steel and the material of the resistance wire is for instance the material that has the product name "cantal". The base 5b consists of an aluminium base and an isolation material that separates the base and the resistance wire so that there cannot occur a short circuit. The resistance wires 3 have been placed into the first holes 3 so that the loops 5a are located in the inside space 6 of the object 100 reaching about half of its height h and the bases 5b are in the first holes 3 leaning with their down side to the collars 3a that there are in these holes. In the second closing means 2 there are provided around the first holes 3 controller sleeves 3b that center the basis 5b of the electric resistances 5 to the middle of the first holes 3 so that the loops 5a have space to penetrate through the first holes 3 to the inside space 6 of the object 100. The bases 5b serve at the same time as the blockers of the first holes 3. The connection cables 5c of the electric resistances 5 are connected to the control unit 7 that has been connected to the electric net 8. Inside 6 the object 100 or near the lining 102 inside the object 100, at least one temperature detector 9 has been installed and it/they are connected using cable 9a or cable free technique to the computer 10. The computer 10 has been connected to the control unit 7 and the computer 10 has a software program that makes it possible that the computer 10 is capable of receiving information from temperature detector 9 and comparing this information with the dry heating plan of the object 100 that has been fed to the computer 10, that is to say the temperature diagram (Fig 1), where the inside temperature of the object 100 or the surface temperature of the lining 102 where the temperature is expressed as the function of time, and the computer 10 is capable of sending information to the control unit 7 whereby the control unit 7 controls the length of the periods of feeding electric power so that the electric energy that is fed to the inside space 6 and that is measured by the temperature detectors 9 follows substantially during the whole drying heating period the temperature diagram of the computer 10 and so that the raising speed of the temperature does not go over and the temperature keeping periods do not go below more than what is accepted in the tolerances, but the process should be as fast as possible. In other words, the lowest temperature value y that the computer 10 receives defines the temperature raising trend t (fig 7) and the temperature keeping start moment x with the condition that at a certain moment the highest temperature value z that the computer 10 uses does not go over constant upper margin m what has been set for it in the time axis to be constant for a certain period of time. It can be said about the fig 7 that in the example it shows the length of the first raising period of the temperature is 1% h longer than the preliminary temperature diagram.

When the dry heating is started the computer 10 is switched on and the control unit 7 is switched on. The temperature diagram shows that the inside lining surface 102c temperature ought to rise with the speed of 20°C per hour until it reaches the temperature of 120°C and on the other hand when the computer 10 receives the information from the temperature detector 9 that at that moment the temperature is constant about 20°C the computer 10 controls with the help of its software program the control unit 7 to connect the electricity to the electric resistances 5. When the temperature that has been registered by the temperature detectors and transmitted to the computer 10 rises faster than what is indicated in the temperature diagram, the control unit cuts the electricity when the margin m has been reached, cuts the electricity from the electric resistances 5 by the command of the computer 10. On and off periods of the electricity follow each other under the cooperation of the computer 10 following the temperature diagram and receiving values from the temperature detectors 9 and the control unit 7 and the temperature of the inside ofobject 100 and the lining layer 102c rises within certain limits following the temperature diagram or more slowly until the desired temperature of 120°C. The raise of the temperature is in practice stepwise but its deviations from the values stated in the temperature diagram are in certain accepted limits. If necessary, the computer program is capable of adding time to the temperature raising periods and their keeping periods, that is to slow down the raising speed of the temperature and to lengthen the keeping periods if the information from some temperature detector means that the lining 102 cannot in all its parts follow the temperature diagram values. Thus we can say that the temperature diagram used in the system is preliminary and the computer software program takes into account all the necessary temperatures of the lining 102 in all moments so that the highest raising temperature is not exceeded and the shortest keeping period of the temperature is not gone below in any part of the lining 102 during the whole dry heating process.

When the inside space 6 of the object 100 and consequently the surface 102c temperature of the lining 102 goes over the 100°C limit the water of the lining 102 starts to evaporate. The temperature is kept in the previous told way sufficiently long at about 120°C and thus all the free water of the construction comes out as steam and leaves the inside space 6 through the other holes 4. The system continues its planned operation with the maximum speed defined in the temperature diagram until the highest temperature of the dry heating (in this example about 550°C) has been reached in all the parts of the surface of the lining 102 and kept the defined period of time. After this, the system cuts the electricity of the electric resistances 5 and the lining 102 of the object 100 cools down slowly back to the temperature of the environment.

The before described raising and keeping of the temperature can also be done so that instead of turning on and of the electricity or in addition to it the amount of the energy fed inside 6 is regulated by change of the power. In this case, a unit that is capable of regulating the power, like for instance a thyristor can be used. One way to reach the same end result is to divide the electric resistances 5 into periods in a different way, a part of the electric resistances can even be turned off completely during the process. The smaller amount of electric resistances are used in the process the longer the periods they are on and the greater the steps to follow the temperature diagram.

In the example that has been described before 12 pcs of 8 kW electric resistances are used and thus the greatest capacity of the process is 96 kW. This capacity is sufficient to obtain the optimum end result. In the system according to the invention the shape of the electric resistance loop 5a can be different than the example e.g. a spiral or some other advantageous shape. In the documents of this application when speaking about the shapes of the electric resistance loops all types of resistance element shapes and constructions are understood. To mention some examples: direct loop, spiral loop and pleat loop.

When making the software program or building the control unit 7 for the system according to this invention very many solutions of the prior-art technique can be applied to attain an advantageous result.

Other advantageous equipments where the system according to this invention can be used are in addition to the previously presented equipment parts and other different parts are whole boilers, kilns, gasifiers, channels, and other equipments containing refractory and isolating ceramic constructions. For instance the dry heating of a boiler furnace or the furnace and cyclone can be performed using the method according to this invention. In that case, the electric resistances would be put into burner openings, man holes or fuel feeding openings. The electric resistances can be placed in different sides of the plant to obtain a more even process. All the other openings are closed with different kind and size of closing means 1, 2 and the gas leaking from the object 100 is eliminated for instance by closing the damper plate. Sufficient paths are arranged for the steam to go out and if possible a closed air circulation is arranged inside the object 100. It is also possible to arrange a closed air circulation in the previous example inside the object 100. In this case, a hole 11 is made in the middle of the second closing means 2 before its installation and into this hole 11 an air ventilator 12 axis 12a is installed. To the outside surface of the second closing means 2, an electric motor 13 is installed and this motor rotates the air ventilator axis 12a. At the other end of the axis 12a, a propeller 12b is installed and its rotation and the propeller blade angle cause a certain type of air circulation in the inside space 6. With this arrangement it is possible to make more effective the process of the inside temperature to become homogenous, so that for example the air near the electric resistances 5 is pushed to the fringes of the inside space 6 and thus the air from the fringes moves closer the electric resistances 5 in the centre of the inside space 6.

When the object 100 of the dry heating is an equipment or its part where the lining 102 of high temperature resistance includes a backside layer or a part thereof made of the castable material and the dry heating must also be performed for this area because of the amount of water it contains, the temperature detector 9 or a number of them is/are placed also in such way that the system gets information also from this part of the construction. The temperature detector is placed exactly to that position in the thickness direction from which position the temperature is desired to be compared to the temperature diagram. In these dry heating processes where there is an isolating castable the processes are self evidently longer than the dry heating of one layer because that background layer sets the speed of the dry heating. In cases like this, the dislocations of the margins m in the time axis can be very big. It is worth noticing that it is not always possible to remove even all the free water from the isolating layer and in those cases one must take this fact into account when placing the temperature detectors. As an example of this kind of case let's mention a lining 102 the utmost isolation layer of which has been done using isolation castable and the shell 101 around the lining 102 has the highest acceptable temperature of less than 100°C in the operation conditions of the plant. Using the system according to the invention it is possible to attain very close the shortest lead-time of the process, because the computer 10 and the control unit 7 run the feed of energy into the inside space 6 without a delay that is always present in hand driven systems.

It is possible to connect to the system according to the invention an automatic alarm system that can tell the end of the process or something else worth noticing.

In those cases where the ceramic lining 102 does not include an isolating material layer, an isolation is installed to the outside surface of the shell 101 of the object 100 in order to minimize the flow of energy through the shell 101 and thus save energy. One material that is typically very suitable for this purpose is rock wool.

It is worth noticing that even though this explanation has kept to one type of example that is advantageous for the system according to the invention the intention is not to limit in any way the use of the invention for only this type of example but many variations are possible within the frames of ideas of the patent claims.

## Claims

1. A method of dry heating of ceramic refractory construction, according to which method:
• The openings of an object (100) to be dry heated like an inside lined boiler, kiln, gasifier or corresponding equipment, the openings like the first opening (104a) and the second opening (104b) are closed using closing means (1,2) that have high temperature proof ceramic surface lids or corresponding closing means (1,2) to obtain a closed inside space (6) inside the object (100),
• the shell (101) of the object (100) is isolated outside using isolation material to prevent the loss of energy if the inside lining (102) does not have an isolating layer and if the object (100) does not have an isolation outside,
• at least one hole is made to lead inside the object (100) for a heating device, this hole is made to the closing means (1,2) or by forming an opening in the object (100) using filler material like for instance ceramic fibre so that the opening is of suitable size,
• at least one hole is made to lead inside the object (100) for steam to come out by making it to the lid, stopper or corresponding closing means (1,2) or forming an opening in the construction to a suitable size using filler material like for instance ceramic fibre,
• at least one heat producing device is installed into an opening made for it or through it into the inside space (6) to heat it for the drying heating of the lining (102) of the object (100),
• at least one temperature detector (9) is installed to the inside space (6) of object (100) and with the help of this/these detector(s) the inside space (6) lining (102) temperature is monitored during the process of the drying heating,
• the air in the inside space (6) and thus also the lining (102) is heated substantially according to a certain temperature diagram in order to get the moisture out of the construction and that the final bonds of the lining (102) can be formed, **characterized in that**:
• at least one heating device is an electric resistance (5) loop (5a) which is pushed through a hole (3) or is installed in some other way in the inside space (6) of the object (100) so that substantially the whole loop (5a) is inside the inside space (6) and the base (5b) of the electric resistance (5) is outside the inside space (6),
• at least one cable (5c) of the electric resistances (5) is connected to a control unit (7) in order to get the necessary energy for the drying heating from the electrical network (8) via the control unit,
• the temperature detector(s) (9) like for instance a detecting element is/are connected by cable or wireless connection to a computer (10) to get the temperature values of the inside space (6) and/or the lining (102) to the computer (10),
• the software program of the computer (10) is started and the program:
o compares the values that come from the temperature detector(s) with the values of the temperature diagram,
o regulates the control unit (7) to increase or decrease the amount of electrical energy to the electric resistances (5) in such a way that the temperature values indicated by the detector(s) in the inside space (6) /the lining (102) remain during the whole process as defined by the preliminary temperature diagram following the raising trends and that keeping periods are not below the defined tolerance, but in any case so that the drying heating process is performed in so fast a period of time than the lowest temperature values (y) allow.

2. The method according to claim 1 **characterized in that** an air ventilator (12) is installed in the inside space (6) like for instance a device consisting of a motor (13), an axis (12a) and a propeller (12b) and this propeller (12b) moves the inside air farther from the electric resistances (5) and thus air from the other parts of the inside space (6) move to the vacuum close the electric resistances (5).

3. The method according to claim 1 or 2 **characterized in that** the amount of the electric power fed to the electric resistance(s)(5) by the control unit (7) is regulated by a thyristor or other corresponding device.

4. The method according to one of the claims 1 to 3 **characterized in that** the electric resistance (5) loop (5a) has an oblong shape.

5. The method according to one of the claims 1 to 4 **characterized in that** an alarm system is connected to it to express that a certain phase has started or ended or something expected or unexpected has happened.

## Patentansprüche

1. Verfahren zum Trocknungswärmen einer feuerfesten Keramikkonstruktion, nach welchem Verfahren:
• Die Öffnungen eines Gegenstands (100), der trocknungsgewärmt werden soll, wie eines innenausgekleideten Boilers, Brennofens, Vergasungsapparats oder von entsprechenden Geräten, die Öffnungen, wie die erste Öffnung (104a) und die zweite Öffnung (104b), verschlossen werden, wobei Verschlusseinrichtungen (1, 2), die hochtemperaturfeste Keramikoberflächen-Deckel aufweisen, oder entsprechende Verschlusseinrichtungen (1, 2) verwendet werden, um einen geschlossenen Innenraum (6) im Innern des Gegenstands (100) zu erzielen,
• der Mantel (101) des Gegenstands (100) unter Verwendung von Isolationsmaterial außen isoliert wird, um den Energieverlust zu verhindern, wenn die Innenauskleidung (102) keine Isolationsschicht aufweist und wenn der Gegenstand (100) außen keine Isolation aufweist,
• mindestens ein Loch für ein Heizgerät so angeordnet wird, dass es ins Innere des Gegenstands (100) führt, dieses Loch an den Verschlusseinrichtungen (1, 2) angeordnet wird oder indem eine Öffnung in dem Gegenstand (100) gebildet wird, wobei Füllmaterial wie beispielsweise Keramikfaser verwendet wird, so dass die Öffnung von geeigneter Größe ist,
• mindestens ein Loch so angeordnet wird, dass es ins Innere des Gegenstands (100) führt, damit Dampf herauskommen kann, indem es am Deckel, Stöpsel oder an entsprechenden Verschlusseinrichtungen (1, 2) angeordnet wird oder indem eine Öffnung in der Konstruktion zu einer geeigneten Größe gebildet wird, wobei Füllmaterial wie beispielsweise Keramikfaser verwendet wird,
• mindestens ein Wärmeerzeugungsgerät in eine dafür hergestellte Öffnung oder durch sie hindurch in den Innenraum (6) eingebaut wird, um es zum Trocknungswärmen der Auskleidung (102) des Gegenstands (100) zu erwärmen,
• mindestens ein Temperaturdetektor (9) am Innenraum (6) von Gegenstand (100) angebracht wird und mit der Hilfe von diesem/diesen Detektor(en) die Innenraum(6)auskleidungs(102)temperatur während des Prozesses des Trocknungswärmens überwacht wird,
• die Luft im Innenraum (6) und folglich auch die Auskleidung (102) im Wesentlichen entsprechend einem gewissen Temperaturdiagramm erwärmt wird, um die Feuchtigkeit aus der Konstruktion zu vertreiben und damit die endgültigen Bindungen der Auskleidung (102) gebildet werden können,
**dadurch gekennzeichnet, dass**:
• mindestens ein Heizgerät eine elektrische Widerstands(5)schleife (5a) ist, die durch ein Loch (3) geschoben wird oder auf eine andere Weise im Innenraum (6) des Gegenstands (100) eingebaut wird, so dass sich im Wesentlichen die ganze Schleife (5a) im Innern des Innenraums (6) befindet und sich die Basis (5b) des elektrischen Widerstands (5) außerhalb des Innenraums (6) befindet,
• mindestens ein Kabel (5c) der elektrischen Widerstände (5) mit einer Steuereinheit (7) verbunden wird, um die notwendige Energie zum Trocknungswärmen von dem Stromnetz (8) über die Steuereinheit geliefert zu bekommen,
• der/die Temperaturdetektor(en) (9), wie z.B. ein Messfühler, durch Kabel oder Funk mit einem Computer (10) verbunden wird/werden, um die Temperaturwerte des Innenraums (6) und/oder der Auskleidung (102) dem Computer(10) zuzuführen,
• das Softwareprogramm des Computers (10) gestartet wird und das Programm:
o die Werte, die von dem/den Temperaturdetektor(en) stammen, mit den Werten des Temperaturdiagramms vergleicht,
o die Steuereinheit (7) so reguliert, dass der Betrag an elektrischer Energie zu den elektrischen Widerständen (5) auf eine solche Weise erhöht oder verringert wird, dass die durch den/die Detektor(en) angezeigten Temperaturwerte in dem Innenraum (6)/der Auskleidung (102) während des gesamten Prozesses so bleiben, wie durch das vorläufige Temperaturdiagramm festgelegt, wobei den Steigerungstendenzen gefolgt wird, und dass sich Halteperioden nicht unterhalb der festgelegten Toleranz befinden, aber auf jedem Fall so, dass der Trocknungswärmprozess in einer so kurzen Zeitspanne erfolgt, als es die niedrigsten Temperaturwerte (y) zulassen.

2. Verfahren nach Anspruch 1, **dadurch gekennzeichnet, dass** ein Luftventilator (12) im Innenraum (6) eingebaut wird, wie beispielsweise ein Gerät, das aus einem Motor (13), einer Achse (12a) und einer Luftschraube (12b) zusammengesetzt ist, und diese Luftschraube (12b) die Innenluft weiter weg von den elektrischen Widerständen (5) bewegt und sich folglich Luft von den anderen Teilen des Innenraums (6) zum Unterdruck in der Nähe der elektrischen Widerstände (5) bewegt.

3. Verfahren nach Anspruch 1 oder 2, **dadurch gekennzeichnet, dass** der Betrag an elektrischer Leistung, die dem/den elektrischen Widerstand (Widerständen) (5) durch die Steuereinheit (7) zugeführt wird, durch einen Thyristor oder ein anderes entsprechendes Bauelement reguliert wird.

4. Verfahren nach einem der Ansprüche 1 bis 3, **dadurch gekennzeichnet, dass** die elektrische Widerstands(5)schleife (5a) eine längliche Form aufweist.

5. Verfahren nach einem der Ansprüche 1 bis 4, **dadurch gekennzeichnet, dass** eine Alarmanlage damit verbunden wird, um zum Ausdruck zu bringen, dass eine gewisse Phase begonnen oder geendet hat oder etwas Erwartetes oder Unerwartetes geschehen ist.

## Revendications

1. Procédé de séchage par la chaleur d'une construction de céramique réfractaire, selon lequel :
• les ouvertures d'un objet (100) à sécher comme une chaudière, un four, un gazéifieur ou un équipement correspondant chemisé interne, les ouvertures comme la première ouverture (104a) et la seconde ouverture (104ab) sont fermées en utilisant des moyens de fermeture (1, 2) qui ont des couvercles de surface en céramique résistant aux températures élevées ou des moyens de fermeture correspondants (1, 2) pour obtenir un espace intérieur clos (6) à l'intérieur de l'objet (100),
• la coque (101) de l'objet (100) est isolée extérieurement en utilisant un matériau d'isolation pour empêcher la perte d'énergie si le chemisage interne (102) n'a pas de couche isolante et si l'objet (100) n'a pas d'isolation extérieure,
• au moins un trou est pratiqué pour conduire à l'intérieur de l'objet (100) destiné à un dispositif de chauffage, ce trou est réalisé dans les moyens de fermeture (1, 2) ou en formant une ouverture dans l'objet (100) en utilisant un matériau de remplissage comme par exemple de la fibre céramique de telle sorte que l'ouverture soit d'une taille convenable,
• au moins un trou est réalisé pour conduire à l'intérieur de l'objet (100) et permettre à la vapeur de s'échapper en pratiquant le trou dans le couvercle, le bouchon ou les moyens de fermeture correspondants (1, 2) ou en formant une ouverture dans la construction ayant une taille convenable en utilisant un matériau de remplissage comme par exemple de la fibre céramique,
• au moins un dispositif producteur de chaleur est installé dans une ouverture prévue à cet effet ou à travers celle-ci pour arriver dans l'espace intérieur (6) afin de le chauffer pour le séchage par la chaleur du chemisage (102) de l'objet (100),
• au moins un détecteur de température (9) est installé dans l'espace intérieur (6) de l'objet (100) et avec l'aide de ce ou de ces détecteurs, la température du chemisage (102) de l'espace intérieur (6) est surveillée durant le processus de séchage par la chaleur.
• l'air dans l'espace intérieur (6) et donc aussi le chemisage (102) est chauffé sensiblement selon un certain diagramme de température afin d'évacuer l'humidité de la construction et de pouvoir former les liaisons finales du chemisage (102),
**caractérisé en ce que** :
• au moins un dispositif de chauffage est une boucle (5a) de résistance électrique (5) qui est poussée à travers un trou (3) ou qui est installée d'une quelconque autre façon dans l'espace intérieur (6) de l'objet (100) de telle sorte que sensiblement toute la boucle (5a) se trouve à l'intérieur de l'espace intérieur (6) et la base (5b) de la résistance électrique (5) se trouve en dehors de l'espace intérieur (6),
• au moins un câble (5c) des résistances électriques (5) est connecté à une unité de commande (7) afin d'obtenir l'énergie nécessaire pour le séchage par la chaleur depuis le réseau électrique (8) par l'intermédiaire de l'unité de commande,
• le ou les détecteurs de température (9) comme par exemple un élément de détection est/sont connectés par câble ou connexion sans fil à un ordinateur (10) afin de fournir les valeurs de température de l'espace intérieur (6) et/ou du chemisage (102) à l'ordinateur (10),
• le programme logiciel de l'ordinateur (10) est lancé et le programme :
○ compare les valeurs qui proviennent du ou des détecteurs de température aux valeurs du diagramme de température,
○ régule l'unité de commande (7) pour augmenter ou diminuer la quantité d'énergie électrique allant aux résistances électriques (5) de telle sorte que les valeurs de température indiquées par le ou les détecteurs dans l'espace intérieur (6)/le chemisage (102) persistent durant tout le processus telles que définies par le diagramme de température préliminaire suivant les tendances à la hausse et que les périodes de maintien ne soient pas inférieures à la tolérance définie, mais dans tous les cas que le processus de séchage soit exécuté dans la période de temps la plus courte possible permise par les valeurs de température (y) les plus basses.

2. Procédé selon la revendication 1, **caractérisé en ce qu'**un ventilateur d'air (12) est installé dans l'espace intérieur (6) comme par exemple un dispositif consistant en un moteur (13), un axe (12a) et une hélice (12b) et cette hélice (12b) éloigne l'air intérieur des résistances électriques (5) et ainsi l'air provenant des autres parties de l'espace intérieur (6) entre dans le vide près des résistances électriques (5).

3. Procédé selon la revendication 1 ou 2, **caractérisé en ce que** la quantité de la puissance électrique alimentée à la ou aux résistances électriques (5) par l'unité de commande (7) est régulée par un thyristor ou autre dispositif correspondant.

4. Procédé selon l'une quelconque des revendications 1 à 3, **caractérisé en ce que** la boucle (5a) de résistance électrique (5) a une forme oblongue.

5. Procédé selon l'une quelconque des revendications 1 à 4, **caractérisé en ce qu'**un système d'alarme lui est connecté pour indiquer qu'une certaine phase a commencé ou s'est achevée ou que quelque chose de prévu ou d'imprévu s'est produit.
